

Patented Dec. 4, 1945

2,390,123

# UNITED STATES PATENT OFFICE

2,390,123

## PRINTING INKS AND VEHICLES THEREFOR

Charles A. Rietz, Park Ridge, and Francis J. Jeuck, Chicago, Ill., assignors to Interchemical Corporation, New York, N. Y., a corporation of Ohio

No Drawing. Application July 22, 1942,  
Serial No. 451,954

11 Claims. (CL 106—30)

This invention relates to printing inks which dry by evaporation of solvent in the vehicle. More particularly, the invention contemplates the provision of an improved printing ink vehicle which will set more effectively when heat is applied to the printed film and which permits even greater speeds of printing and greater economy in the printing process.

Ordinary linseed oil inks dry by oxidation of the ink vehicle and consequently cannot be printed at the high speeds demanded today even when various driers are included in the ink. At present, such inks are primarily used in sheet-fed presses, and it is necessary to use slip sheets and/or offset-preventing powders to prevent the transfer of the freshly printed ink from one sheet to the next; and in some cases heat is used to accelerate the drying.

The problem of high speed printing on other than porous stock was solved with the introduction of the inks disclosed in A. E. Gessler Patent No. 2,087,190, dated July 13, 1937. These inks consist of pigment dispersed in a vehicle comprising binder dissolved in a solvent which is not volatile at normal room temperatures (about 70° F.), but which evaporates rapidly when heated to elevated temperatures (about 240° F.). Inks of this character are quickly and effectively dried by passing them through an oven which may be heated by means of open flames so that the solvent vapors will be burned. However, due to the amount of heat required to dry the solvent inks that are now available, the cost of heating is an important consideration in the ultimate cost of the printing process. Furthermore, there are many kinds of paper upon which the intense heat required for effective drying has an undesirable effect. In addition, attempts are constantly being made to increase the speed and decrease the cost of the printing process.

We have discovered a new and improved printing ink of the binder-solvent type which permits increased speeds in the printing process at less cost than is possible with inks heretofore available. This new ink comprises pigment dispersed in a vehicle consisting of resin dissolved in a solvent which is substantially non-volatile at ordinary room temperatures (about 70° F.), but which evaporates rapidly when heated to elevated temperatures (about 240° F.), said vehicle having a small percentage (about 1/2 to 6%) of a film-forming agent colloidally distributed throughout the vehicle. The film-forming agent is characterized by the fact that it is at least largely insoluble in the ink vehicle at ordinary temperatures, and at elevated temperatures well below its fusion point, but becomes more soluble in the vehicle as the solvent is lost.

The improved results are obtained when small percentages (from 0.5 to 6% of the ink vehicle)

of a completely insoluble film-forming agent are distributed in colloidal form throughout the vehicle. However, film-forming agents which are partially soluble in the ink vehicle are most often used; in such event, the total amount present in the vehicle will be such as to produce saturation of the vehicle, plus an additional insoluble percentage in the indicated range, distributed in colloidal form throughout the vehicle.

10 It is important to have the film-forming agent distributed in colloidal form through the vehicle. If the agent is not in colloidal form, or if more than about 6% of it is present in the vehicle in colloidal form, poor printing results, particularly in half-tone work.

15 The added film-forming agent, being insoluble in the solvent and vehicle, has little effect on the body of the ink at printing temperatures and concentrations. However, as the concentration of 20 resin (which is apparently a solvent for the film-forming agent) goes up, on evaporation of solvent, the film-forming agent goes increasingly into solution; the solution of resin, solvent and film-forming agent is far stiffer than the resin-solvent mixture alone, and thus we obtain enhanced drying.

25 Even better results are obtained, in heat-drying, where sufficient insoluble film-forming agent is present so that it does not go completely into 30 solution on evaporation of the solvent. Apparently the colloidally distributed insoluble material substantially reduces the stickiness of the film, probably acting as an offset preventing medium, and perhaps as an adsorbent. This effect is substantial enough so that enhanced heat-drying can be obtained even when completely insoluble 35 film-forming agents are used, as described in our co-pending application Serial No. 451,764, filed July 21, 1942.

40 To obtain the desired colloidal distribution of the small percentage of film-forming agent, more than mere stirring, mixing, or grinding of the agent in powder form into the vehicle is desirable. We have found that the colloidal distribution can 45 be obtained by heating the vehicle, with the film-forming agent added thereto, to a temperature above the melting point of the film-forming agent and maintaining the mixture at that temperature for a period sufficient to melt the film-forming agent. Then upon cooling of the vehicle to room 50 temperature the film-forming agent separates out of the mixture to form the desired colloidal suspension. It is also possible to obtain the proper colloidal distribution by dissolving the film-forming agent in a solvent, adding the solution to the ink vehicle to obtain a uniform mixture, and then evaporating the solvent, preferably while grinding the ink, so that the film-forming agent separates out of the ink in colloidal form. A third 55 method comprises malaxation of the insoluble 60 method comprises malaxation of the insoluble

film-forming ingredient with the resin, followed by cutting with the solvent. Typical examples of printing ink vehicles embodying the principles of our invention and compounded in accordance with our preferred procedure are as follows:

*Example 1*

Parts by weight

|                                                                                                                                        |      |
|----------------------------------------------------------------------------------------------------------------------------------------|------|
| Solvent (petroleum cut, having a distillation range of 5% at 497° F. and 95% at 527° F., having a dimethyl sulfate value of 3.0) _____ | 1320 |
| F' gum rosin _____                                                                                                                     | 1630 |

These are melted together in an open kettle at a temperature of 350° F., and after melting add slowly, allowing time for reaction between additions:

Lime \_\_\_\_\_ 106

When reaction is completed and foam is down, add—

Ethyl cellulose (20 centipoise, high ethoxy content) \_\_\_\_\_ 130

Close kettle and heat to 410° F., holding at that temperature for two hours. After cooling, add—

Solvent (petroleum cut, having a distillation range of 5% at 497° F. and 95% at 527° F., having a dimethyl sulfate value of 3.0) \_\_\_\_\_ 900

\_\_\_\_\_ 4096

In this limed rosin varnish, the film-forming agent is ethyl cellulose and constitutes about 3.2% of the total varnish, some of which goes into solution, but the majority of which is distributed in colloidal form throughout the varnish. This varnish has a mushy consistency due to the colloidal distribution of ethyl cellulose. However, one pass on a three-roller mill renders it free-flowing.

Inks made from this vehicle print well, and can be dried much more rapidly than similar inks without the ethyl cellulose added. The amount of ethyl cellulose used is sufficient to more than saturate the vehicle at dryness—hence, the added drying effect of the distributed ethyl cellulose can be observed here.

*Example 2*

Parts by weight

|                                                                                                                                     |      |
|-------------------------------------------------------------------------------------------------------------------------------------|------|
| Solvent (petroleum cut, having a distillation range of 5% at 475° F. and 95% at 500° F., and a dimethyl sulfate value of 2.5) _____ | 1000 |
| F' gum rosin _____                                                                                                                  | 2200 |

Melt at 350° F., and add slowly:

Lime \_\_\_\_\_ 145

When reaction is complete, add—

Ethyl cellulose (20 centipoise, high ethoxy content) \_\_\_\_\_ 52

Heat to 410° F. and hold at that temperature for only 30 minutes. When cooled, add—

Solvent (petroleum cut, having a distillation range of 5% at 475° F. and 95% at 500° F., and a dimethyl sulfate value of 2.5) \_\_\_\_\_ 800

\_\_\_\_\_ 4197

In this example, the ethyl cellulose only constitutes about 1.2% of the total varnish. Most of this is insoluble in the vehicle under printing con-

ditions, but becomes soluble under drying conditions.

*Example 3*

Pounds

|                                          |     |
|------------------------------------------|-----|
| 5 Terpene-phenol resin (Durez 220) _____ | 450 |
| and                                      |     |

|                                                                                                                            |     |
|----------------------------------------------------------------------------------------------------------------------------|-----|
| Solvent (petroleum distillate—distillation range of 5% at 513° F. and 95% at 542° F., dimethyl sulfate value of 3.0) _____ | 450 |
|----------------------------------------------------------------------------------------------------------------------------|-----|

are refluxed at 410-420° F. until the resin is dissolved.

|                                                                |    |
|----------------------------------------------------------------|----|
| 15 Ethyl cellulose (20 centipoise—medium ethoxy content) _____ | 45 |
|----------------------------------------------------------------|----|

are then added, and the mass held at 410-420° F. for 30 minutes

|               |    |
|---------------|----|
| Solvent _____ | 35 |
|---------------|----|

20 are then added.

This vehicle shows a most pronounced change in solubility as solvent is lost and resin solids increase. However, a small percentage of insoluble ethyl cellulose generally remains to add to the effect of that which goes into solution.

An example of an ink made with one of the vehicles described above is as follows:

*Example 4*

Parts by weight

|                                                      |      |
|------------------------------------------------------|------|
| Varnish of Example 3, or of the other examples _____ | 1030 |
| Stearine pitch _____                                 | 60   |

|                                                                                                                                             |     |
|---------------------------------------------------------------------------------------------------------------------------------------------|-----|
| 35 Solvent (petroleum cut, having a distillation range of 5% at 497° F. and 95% at 527° F., and having a dimethyl sulfate value of 6) _____ | 150 |
|---------------------------------------------------------------------------------------------------------------------------------------------|-----|

|                       |     |
|-----------------------|-----|
| Inert extenders _____ | 70  |
| Carbon black _____    | 520 |

|                              |    |
|------------------------------|----|
| 40 Prussian blue toner _____ | 50 |
|------------------------------|----|

The above were mixed well on a four roller mill, and then—

|                            |     |
|----------------------------|-----|
| Varnish of Example 1 _____ | 800 |
|----------------------------|-----|

45 were added and mixing completed.

\_\_\_\_\_ 2680

This produced a black ink which dried rapidly and without offset at web speeds of about 1200-1400 feet per minute.

Obviously, other pigments, fillers and ingredients conventionally used in inks (waxes, soaps, wetting agents, etc.) can be used to replace those indicated.

While the examples are restricted to various grades of ethyl cellulose, other film-forming agents which exhibit the desired solubilities can be used. Thus, we have used nitrocellulose with alkyd resins which have a solvent action thereon; and other cellulose esters and ethers, and various resins, can all be used.

While the invention is particularly applicable to heat-drying inks, it is obviously applicable in hastening the drying of any resin-solvent film-forming composition, whether air-dried or heat-dried.

We claim:

1. A typographic printing ink vehicle comprising a solution of a resin in a solvent therefor, which is substantially non-volatile at 70° F., but which evaporates rapidly when heated to temperatures of the order of 240° F., having a small percentage of a film-forming agent distributed in colloidal form therethrough, said small per-

centage of film-forming agent comprising from 0.5 to 6%, based on total vehicle weight, of material insoluble in the solvent and the resin solution at normal room temperatures, but becoming increasingly soluble as the resin concentration of the solution increases by removal of solvent, whereby the film obtained from the ink is further advanced in dryness by solution of the film-forming agent.

2. A typographic printing ink vehicle comprising a solution of a resin in a hydrocarbon liquid substantially volatile at 70° F., but rapidly volatile at temperatures of the order of 240° F., having a small percentage of a film-forming agent distributed in colloidal form therethrough, said 15 small percentage of film-forming agent comprising from 0.5 to 6%, based on total vehicle weight, of material insoluble in the solvent and the resin solution at normal room temperatures, but becoming increasingly soluble as the resin concentration of the solution increases by removal of solvent, whereby the film obtained from the ink is further advanced in dryness by solution of the film-forming agent.

3. A printing ink vehicle comprising a solution of a resin in a hydrocarbon liquid substantially non-volatile at 70° F., but which evaporates rapidly when heated to temperatures of the order of 240° F., having a small percentage of a film-forming agent distributed in colloidal form therethrough, a portion of said film-forming agent being soluble in the resin solution, but a portion thereof, from 0.5 to 6%, based on total vehicle weight, being insoluble in the solvent and the resin solution at normal room temperatures, but becoming increasingly soluble as the resin concentration of the solution increases by removal of solvent, whereby the film obtained from the ink is further advanced in dryness by solution of the film-forming agent.

4. A typographic printing ink vehicle comprising limed rosin dissolved in a low solvency petroleum hydrocarbon substantially non-volatile at 70° F., but rapidly volatile at temperatures of the order of 240° F., the vehicle having from 0.5 to 6% of ethyl cellulose dispersed through the vehicle in colloidal form, a substantial portion of said ethyl cellulose being insoluble in the solvent and the resin solution at normal room temperatures, but becoming increasingly soluble as the resin concentration of the solution increases by removal of solvent, whereby the film obtained from the ink is further advanced in dryness by solution of the film-forming agent.

5. A typographic printing ink vehicle comprising terpene phenol resin dissolved in a low solvency petroleum hydrocarbon substantially non-volatile at 70° F., but rapidly volatile at temperatures of the order of 240° F., the vehicle having from 0.5 to 6% of ethyl cellulose dispersed through the vehicle in colloidal form, a substantial portion of said ethyl cellulose being insoluble in the solvent and the resin solution at normal room temperatures, but becoming increasingly soluble as the resin concentration of the solution increases by removal of solvent, whereby the film obtained from the ink is further advanced in dryness by solution of the film-forming agent.

6. A printing ink vehicle comprising a solution of a resin in a solvent therefor which is substantially non-volatile at 70° F., but rapidly volatile at temperatures of the order of 240° F., together with another film-forming agent, the film-forming agent being slightly soluble in the resin solution, being present in quantity from 0.5 to 6%, based on total vehicle weight, above that required to saturate the resin solution, said excess being distributed in colloidal form in the solution, the film-forming agent being characterized by its increased solubility in the resin solvent combination as the percentage of resin increases.

7. A printing ink vehicle comprising a solution of a resin in a solvent therefor which is substantially non-volatile at 70° F., but rapidly volatile at temperatures of the order of 240° F., together with another film-forming agent, the film-forming agent being slightly soluble in the resin solution, being present in quantity from 0.5 to 6%, based on total vehicle weight, above that required to saturate the resin solution, said excess being distributed in colloidal form in the solution, the

25 film-forming agent being characterized by its increased solubility in the resin solvent combination as the percentage of resin increases, but not of such greatly increased solubility that it is completely dissolved in the resin solution when a film thereof is set to the touch.

8. A printing ink comprising pigment dispersed in the vehicle of claim 2.

9. A printing ink comprising pigment dispersed in the vehicle of claim 6.

35 10. A heat-drying ink comprising pigment dispersed in a vehicle comprising essentially a solution of limed rosin in a petroleum hydrocarbon liquid which is a non-solvent for high ethoxy ethyl cellulose and is substantially non-volatile at 70° F., but rapidly volatile at 240° F., having col-

lloidally dispersed therein from 0.5 to 6% of high ethoxy ethyl cellulose, the proportion of limed rosin to hydrocarbon being such that the ethyl cellulose is insoluble in the resin solution at normal room temperatures, but becoming increasingly soluble as the resin concentration of the solution increases by removal of solvent, whereby the film obtained from the ink is further advanced in dryness by solution of the ethyl cellulose.

55 11. A heat-drying printing ink comprising pigment dispersed in a vehicle comprising essentially a solution of a terpene phenolic resin in a petroleum hydrocarbon liquid which is a non-solvent for ethyl cellulose and is substantially non-volatile at 70° F., but rapidly volatile at 240° F., having colloidally dispersed therein from 0.5 to 6% of ethyl cellulose, the proportion of terpene phenolic resin to hydrocarbon being such that the ethyl cellulose is insoluble in the resin solution at normal room temperatures, but becoming increasingly soluble as the resin concentration of the solution increases by removal of solvent, whereby the film obtained from the ink is further advanced in dryness by solution of the ethyl cellulose.

CHARLES A. RIETZ.  
FRANCIS J. JEUCK.